

# UNITED STATES PATENT OFFICE.

FELIX FREMERAY, OF NEWARK, NEW JERSEY.

## ART OF MANUFACTURING CLOTH FROM ANIMAL AND VEGETABLE FIBERS.

SPECIFICATION forming part of Letters Patent No. 307,713, dated November 4, 1884.

Application filed February 6, 1883. (No specimens.)

*To all whom it may concern:*

Be it known that I, FELIX FREMERAY, formerly of Aix-la-Chapelle, Germany, but now a resident and about to become a citizen of 5 Newark, New Jersey, United States of America, have invented a certain new and useful Art of Manufacturing Cloth From Mixed Animal and Vegetable Fibers, of which the following is a specification.

10 The object of my invention is to improve the process of producing a cloth of mixed vegetable fiber such as is obtained from ramie, china-grass, or other stalks or blades and animal fiber treated in such manner, substantially as hereinafter particularly set forth and 15 claimed, as to produce a cloth of substantially the same appearance as an all-wool cloth, but which is cheaper and stronger.

In practicing my invention I treat the animal fiber in any usual way by greasing or soap- 20 ing it, and then add to it the vegetable fiber, as much as fifty per centum, and then proceed to spin the mixed fibers in the usual way. I do not oil or grease or soap the vegetable fiber, 25 as I find such substances cause it to curl and become knotty; but I introduce the vegetable fiber in a dry state, free from oil or soap. The yarn spun from such mixed fiber is then woven in the usual way and the cloth subjected to the 30 ordinary washing and fulling processes. As the vegetable fiber does not work up well if "teased" in the wet state, the cloth is twice teased, first, while it is still wet from the wash-

ing, to improve the animal fiber; and, second, after this first teasing and a subsequent dry- 35 ing, to improve the vegetable fiber. This teasing twice—once while wet for the improvement of the animal fiber and once while dry for the improvement of the vegetable fiber—is of great importance in giving a fine woolly surface to 40 the fabric. Ramie, like many other vegetable fibers, is much stronger than animal fibers, and hence a cloth comprising such fibers in admixture will be much stronger than an all-wool fabric. By my improved process of making cloth 45 of such combined fibers I obtain a fabric very closely resembling in touch, look, and color an all-wool cloth, and at the same time far stronger and cheaper. Such a cloth can be made of one-half wool and one-half ramie; but the proportions may be varied with this and other 50 combinations to suit the manufacturer.

What I claim is—

The improved process of producing a cloth of mixed animal and vegetable fibers, the same 55 consisting in oiling or soaping the animal fiber, then mixing therewith the vegetable fiber, spinning the mixed fibers and weaving the same into cloth as usual, washing the cloth, and then teasing it while wet, and drying the 60 cloth and again teasing it while dry, substantially as described.

FELIX FREMERAY.

In presence of—

J. C. CLAYTON,

CHARLES HOLZHAUER.